

# United States Patent Office

3,117,924

Patented Jan. 14, 1964

1

3,117,924

## FLOTATION PROCESS TO PRODUCE SEPARATE ALUMINUM SILICATES AND ZIRCON CONCENTRATES FROM A HEAVY MINERAL BEACH SAND CONCENTRATE

Robert E. Baarson, La Grange, and Charles W. Jonaitis, Chicago, Ill., assignors to Armour and Company, Chicago, Ill., a corporation of Delaware

No Drawing. Filed Dec. 16, 1960, Ser. No. 76,131

6 Claims. (Cl. 209—166)

This invention relates to a method for concentrating the aluminum silicates and zircon in sand deposits which are usually known as beach sands. More particularly this invention relates to a method for making a bulk separation of the aluminum silicates and zircon from a non-magnetic, non-conductive fraction of beach sand concentrate.

Beach sands of the type with which the present invention is concerned may be found along the seashore, but are also found in large inland deposits in Florida and elsewhere. These sand beds or deposits are composed principally of quartz, while containing a small proportion of valuable minerals, among them being titanium oxide minerals like ilmenite and rutile, as well as other heavy minerals such as kyanite-sillimanite, zircon, staurolite, and dumortierite. Usually the content of quartz in these sands will be at least 90% while the content of the various heavy minerals may vary from a trace to upwards of 4%.

The most valuable product at the present time derived from these beach sands is the titanium oxide minerals. These and other conductive and magnet-responsive heavy minerals are being recovered from beach sand deposits by complicated and expensive procedures. For example, the steps in one of these processes involves passing the beach sands through a series of spiral concentrators to make a rough separation of the titanium oxide and other heavy minerals from the quartz. Following the rougher separation, there are cleaner and recleaner spiral circuits to upgrade the rough concentrate, and a large amount of the middling material is recycled through these circuits to increase recovery. The titanium minerals in the heavy mineral concentrate are then further separated and concentrated by electrostatic and magnetic separators. The electrostatic separation removes the ilmenite and rutile while induced roll magnets are employed to remove the staurolite and dumortierite.

The resultant non-conductive, non-magnetic reject fractions from this operation contain minerals which are in themselves valuable. The composition of this beach sand concentrate ore is approximately 40 to 50% aluminum silicates, also referred to as the kyanite-sillimanite fraction, 20 to 30% zircon, and 25 to 40% quartz. It is with these fractions that the present invention is principally concerned.

The problem involved in using such ores to obtain an aluminum silicates and zircon product of high grade in economically feasible recoveries has heretofore received little attention. The industry has always realized that this discarded material contained valuable heavy minerals but no commercially feasible method has up to now been devised to obtain the minerals in the proper grade and recovery. Applicants have solved the problem and have provided through this invention a flotation method which enables the bulk concentration of the valuable aluminum silicate and zircon fractions from the non-magnetic, non-conducting fraction of beach sand concentrates.

It is therefore a general object of this invention to provide a method for concentrating the aluminum silicates and zircon in beach sands, and specifically, to

2

provide a flotation method for accomplishing this result from preprocessed beach sand concentrates. More specifically, it is an object of this invention to provide a flotation method by means of which the aluminum silicates and zircon in preprocessed beach sands can be separated from the quartz particles of such sands. It is also an object of this invention to provide means for carrying out a bulk separation of the aluminum silicates and zircon in beach sand from the quartz and then, in turn to provide means for carrying out a bulk separation of the aluminum silicates from the zircon. Further objects and advantages of this invention will appear as the specification proceeds.

In practicing the present invention, the beach sand fraction from which the titanium oxide minerals have been separated is formed into a flotation feed. The particles of this fraction as received range from —30 to +200 mesh.

Although it is not generally necessary to pretreat the feed, some scrubbing and desliming may be necessary to remove clay minerals and other materials from those ores used in the process that contain them. The feed is conditioned directly with an anionic collector. An auxiliary collector such as crude fuel oil and a frother such as pine oil may be added. The use of either an auxiliary collector, which may also act as a froth modifier, and a frother is optional and may be omitted.

Following conditioning of the feed, the pulp is diluted to form an aqueous slurry containing from 10 to 30% solids. To this slurry of flotation feed is added a fluorine containing acid or a mineral acid such as sulfuric acid, or a combination thereof, and the pH of the aqueous feed is adjusted to a pH below about 6.0 and preferably below about 3.0. Then the quartz is depressed by the acid employed and is passed out in the underflow from the cells. The froth product obtained from the flotation operation is made up mainly of the aluminum silicates and the zircon.

The froth product is then preferably scrubbed with a suitable agent such as sodium hydroxide or potassium hydroxide. Specifically, an aqueous slurry of the froth product is formed and from 1 to 2 pounds per ton of caustic is added per ton of product. This slurry or pulp is mixed until the anionic collector employed in the initial separation operation has been removed from the aluminum silicate and zircon particles. This usually takes from 3 to 5 minutes.

The thus prepared pulp may then be conditioned at an alkaline pH with an amine collector in the presence of a depressant selected from the group consisting of dextrans, gums, and starches. Again employing conventional flotation procedures the zircon concentrate is obtained in the overflow leaving an aluminum silicates concentrate in the tailing.

Various anionic collectors may be employed to float the aluminum silicates and zircon from the quartz particles. However, to obtain an aluminum silicate and zircon concentrate of high grade in economically practical recoveries, it is preferred to use as a collecting agent a compound selected from the group consisting of alpha sulfo fatty acids, the alkali metal salts of such acids, the glyceryl and glycol esters of the acids, sulfonated oils and the alkali metal salts of such oils. Examples of preferred compounds are alpha sulfo stearic acid, alpha sulfo palmitic acid, the sodium or potassium salts of these compounds, the beta-hydroxyethylene ester of alpha sulfo stearic acid, the mono and di ethylene glycol esters of alpha sulfo stearic and palmitic acids, sulfonated glyceride oils and petroleum oils, and mahogany sulfonates.

To achieve the outstanding results of the present invention it is only necessary to add small quantities of the

collecting agent to the ore. Usually from 0.1 to about 4.0 pounds of the agent per ton of ore will be satisfactory, with from 0.2 to 1.0 pounds per ton being preferred.

The fluorine containing acid which is used as a depressant is preferably hydrofluoric acid although other fluorine containing acids can be substituted, as well as mixtures of hydrofluoric acid and other fluorine containing acids.

The pH of the flotation slurry in separating the aluminum silicates and zircon from the quartz should not exceed about pH 6.0. Best results are achieved at a pH below 3.0. Part of the necessary hydrogen ion concentration to achieve the desired pH can be supplied by the fluorine containing acid, but for economic reasons it will usually be preferred to use an additional acid, such as sulfuric or hydrochloric acid to maintain the flotation circuit at an acid pH.

In bringing about the separation of the aluminum silicates from the zircon concentrate, any amine collector may be employed. Preferably, however, the amine flotation agent is a primary amine containing a hydrophobic group of from 6 to 22 carbon atoms. Mixed amines like primary tallow and soya amines are suitable. Best results are achieved when the amine flotation agent is used in the form of a water-soluble salt thereof, such as an amine acetate or hydrochloride salt. Both monoamines and polyamines can be used in addition to certain quaternary compounds such as dialkyl dimethyl quaternary ammonium chloride, sulfate, etc.

The pH of the flotation feed in separating the aluminum silicates from the zircon is usually carried out at an alkaline pH in the range from 7.0 to 12.0 and preferably in the range from 8.0 to 10.0. Since the present invention does not depend for its success on the choice any specific base material, any suitable base may be employed to provide the desired pH. Examples of such bases are sodium hydroxide, potassium hydroxide, sodium carbonate, and the like.

The depressant employed in effecting a separation of the aluminum silicates from the zircon may, as indicated, be selected from the group consisting of dextrans, gums

and starches. These agents have the effect of depressing the aluminum silicates permitting the zircon to be obtained as the froth product.

In practicing this invention it is preferred to employ a frothing agent to float the various concentrates. Examples of suitable frothers are pine oil and Dowfroth 250. Similarly, it has been found desirable to use a frothing modifier such as kerosene, fuel oil, diesel oil or other petroleum distillates. Such agents have the effect of suppressing the amount of froth while serving the function of what is believed to be a secondary collector for the aluminum silicates and zircon.

The pulp density in the conditioning and flotation circuits may be varied widely. In the conditioning circuit the solids may be as low as 25%. However, 60 to about 85% solids is preferred and 70% solids is considered an optimum condition. In the flotation circuit the solids may run as high as 40% and as low as 10%. A 25% pulp density, however, is especially effective for flotation.

The flotation operations themselves may be carried out in the usual type of flotation cells provided with means for supplying air to the lower portion of the cells. When the beach sand concentrate has been treated and conditioned as described and the flotation feed is at the desired pH, the aluminum silicates and zircon can be readily floated away from the quartz. In other words, the aluminum silicates and the zircon will be recovered in the overflow from the cells, while the quartz will be depressed and will pass out in the underflow from the cells. Similarly, the aluminum silicates and zircon concentrates, employing the material described and conditions specified, may be separated with conventional equipment.

This invention is further described in the following specific examples:

EXAMPLE I  
Preparation of ore \_\_\_\_ Condition ore at 85% solids for 1 minute with 0.25 lb./ton alpha-sulfo stearic acid, then for 1 minute with 0.5 lb./ton crude fuel oil.  
Flotation machine \_\_\_\_ Fagergren.  
Water \_\_\_\_ Distilled.  
Temperature \_\_\_\_ 25° C.

#### REAGENTS AND CONDITIONS

| Point of Addition                                                                      | Time Cond         | Float (Min.)                 | Percent Solids | pH  | Alpha-Sulfo Stearic Acid | Crude Fuel Oil | HF (48%) | NaOH | Dextrin 164 | Armac T | Pine Oil |
|----------------------------------------------------------------------------------------|-------------------|------------------------------|----------------|-----|--------------------------|----------------|----------|------|-------------|---------|----------|
| 1st Rougher                                                                            | {<br>1/4<br>2 1/4 | 85<br>20<br>*2.8 I<br>*2.9 F | 0.25           | 0.5 |                          | 1.06           |          |      |             |         |          |
| Scrub 1st Rougher for 5 minutes at 20% solids with 2.0 lb./ton NaOH, deslime and wash. |                   |                              |                |     |                          |                |          |      |             |         |          |
| 1st Zircon Concentrate                                                                 | {<br>1/4<br>2 1/4 | 9.4 I<br>6.9 F               |                |     |                          |                |          | 0.08 | 2.0         | 0.3     | 0.34     |
| 2nd Zircon Concentrate                                                                 | {<br>1/4<br>1     | 8.9 I<br>6.9 F               |                |     |                          |                |          | 0.04 | 0.2         | 0.17    |          |

\*I—Initial, F—Final.

REMARKS.—Alpha sulfo stearic acid used as a 10% solution in water, crude fuel oil used is No. 6 grade Bunker "C" fuel oil—Dextrin 164 obtained from Corn Products—1 and 2 Zircon concentrates combined for analysis—Armac T is an acetate salt of a tallow amine.

#### METALLURGICAL RESULTS

| Product                  | Weight Grams | Weight Percent | Percent Heavy Minerals <sup>1</sup> | Percent Grade <sup>2</sup> | Percent Recovery <sup>2</sup> |
|--------------------------|--------------|----------------|-------------------------------------|----------------------------|-------------------------------|
| Quartz Conc.             | 170          | 34.1           | 10.4                                |                            |                               |
| Zircon Conc.             | 114          | 22.9           | 99.25                               | 87.7                       | 76.1                          |
| Aluminum Silicates Conc. | 214          | 43.0           | 99.68                               | 86.7                       | 85.8                          |
|                          | 498          |                |                                     |                            |                               |

<sup>1</sup> Percent Heavy Minerals attained by heavy media separation.

<sup>2</sup> Grade and Recovery obtained by petrographic analysis.

**5**  
**EXAMPLE II**

**6**

Preparation of ore ---- Condition ore at 85% solids for 1 minute with 0.50 lb./ton alpha-sulfo lauric acid, then for 1 minute with 0.5 lb./ton crude fuel oil.

Flotation machine ---- Fagergren.  
Water ----- Distilled.  
Temperature ----- 25° C.

5

**REAGENTS AND CONDITIONS**

| Point of Addition | Time Cond. | Float (Min.) | Percent Solids             | pH | Alpha-Sulfo Lauric Acid | Crude Fuel Oil | H <sub>2</sub> F (48%) | H <sub>2</sub> SO <sub>4</sub> | NaOH | Dextrin 164 | Duomac C | Pine Oil |
|-------------------|------------|--------------|----------------------------|----|-------------------------|----------------|------------------------|--------------------------------|------|-------------|----------|----------|
| 1st Rougher       | {<br>1/4   | 2 1/4        | 85<br>20<br>2.9 I<br>2.9 F |    | 0.5                     | 0.5            | 0.26                   | 0.6                            |      |             |          |          |
|                   |            |              |                            |    |                         |                |                        |                                |      |             |          |          |

Scrub 1st Rougher for 5 minutes at 20% solids with 2.0 lb./ton NaOH, deslime and wash.

|                        |          |       |                |  |  |  |  |      |  |     |      |      |
|------------------------|----------|-------|----------------|--|--|--|--|------|--|-----|------|------|
| 1st Zircon Concentrate | {<br>1/4 | 2 1/4 | 9.5 I<br>6.9 F |  |  |  |  | 0.08 |  | 2.0 | 0.1  | 0.17 |
| 2nd Zircon Concentrate | {<br>1/4 | 1     | 9.0 I<br>7.0 F |  |  |  |  | 0.04 |  | 0.2 | 0.17 |      |

REMARKS.—Alpha-sulfo lauric acid used as a 10% solution in water. Crude fuel oil used is No. 6 Bunker "C" fuel oil. Dextrin 164 obtained from Corn Products 1st and 2nd Zircon Concentrate combined for analysis. Duomac C is a diacetate salt of a coco diamine.

**METALLURGICAL RESULTS**

| Product                  | Weight, Grams | Weight, Percent | Percent Heavy Minerals | Percent Grade | Percent Recovery |
|--------------------------|---------------|-----------------|------------------------|---------------|------------------|
| Quartz Cone              | 149           | 30.1            | 3.52                   |               |                  |
| Zircon Conc.             | 186           | 37.5            | 96.76                  | 62.0          | 91.1             |
| Aluminum Silicates Conc. | 161           | 32.4            | 99.64                  | 94.7          | 69.0             |
|                          | 496           |                 |                        |               |                  |

**EXAMPLE III**

Preparation of ore ---- Condition ore at 85% solids for 1 minute with 0.25 lb./ton mono-ethylene glycol ester of alpha sulfo stearic acid, then for 1 minute with 0.5 lb./ton crude fuel oil.

Flotation machine ---- Fagergren.  
Water ----- Distilled.  
Temperature ----- 25° C.

**REAGENTS AND CONDITIONS**

| Point of Addition | Time Cond. | Float (Min.) | Percent Solids             | pH | Monoethylene glycol ester of Alpha-Sulfo Stearic Acid | Crude Fuel Oil | H <sub>2</sub> F (48%) | NaOH | Dextrin 164 | Armac T | Pine Oil |
|-------------------|------------|--------------|----------------------------|----|-------------------------------------------------------|----------------|------------------------|------|-------------|---------|----------|
| 1st Rougher       | {<br>1/4   | 2 1/4        | 85<br>20<br>2.8 I<br>2.9 F |    | 0.25                                                  | 0.5            | 1.96                   |      |             |         |          |
|                   |            |              |                            |    |                                                       |                |                        |      |             |         |          |

Scrub 1st Rougher for 5 minutes at 20% solids with 2.0 lb./Ton NaOH, deslime and wash twice

|                        |          |       |                |  |  |  |  |       |     |     |      |
|------------------------|----------|-------|----------------|--|--|--|--|-------|-----|-----|------|
| 1st Zircon Concentrate | {<br>1/4 | 2 1/4 | 7.6 I<br>6.3 F |  |  |  |  | trace | 2.0 | 0.2 | 0.17 |
| 2nd Zircon Concentrate | {<br>1/4 | 1     | 7.7 I<br>6.4 F |  |  |  |  |       | 0.2 | 0.2 | 0.17 |

REMARKS.—Monoethylene glycol ester of alpha-sulfo stearic acid used as a 10% solution in water. Crude fuel oil used is No. 6 grade Bunker "C" fuel oil. 1st and 2nd Zircon concentrates combined for analysis. Armac T is an acetate salt of a tallow amine.

**METALLURGICAL RESULTS**

| Product                  | Weight, Grams | Weight, Percent | Percent Heavy Minerals | Percent Grade | Percent Recovery |
|--------------------------|---------------|-----------------|------------------------|---------------|------------------|
| Quartz Cone              | 161           | 32.3            | 8.10                   |               |                  |
| Zircon Conc.             | 174           | 34.9            | 97.73                  | 58.1          | 83.2             |
| Aluminum Silicates Conc. | 164           | 32.8            | 99.53                  | 87.9          | 64.1             |
|                          | 499           |                 |                        |               |                  |

7  
EXAMPLE IV

Preparation of ore ---- Condition ore at 85% solids for 2 minutes with 0.25 lb./ton di-sodium alpha sulfo stearate, then for 1 minute with 0.5 lb./ton crude fuel oil.

Flotation machine ---- Fagergren.  
Water ----- Distilled.  
Temperature ----- 25° C.

5 from the aluminum silicates in a second aqueous medium containing an amine collector and a depressant selected from the group consisting of dextrans, gums and starches, said second aqueous medium having been adjusted to a pH of from 7.0 to 12.0 for said separation.

6 2. The process as claimed in claim 1 wherein the anionic collector is alpha sulfo stearic acid.

## REAGENTS AND CONDITIONS

| Point of Addition | Time Cond.      | Float (Min.)  | Percent Solids | pH             | Di-Na Alpha-Sulfo Stearate | Crude Fuel Oil | HF (48%) | NaOH | Starch 3366 | Armac T | Pine Oil |
|-------------------|-----------------|---------------|----------------|----------------|----------------------------|----------------|----------|------|-------------|---------|----------|
| 1st Rougher       | { $\frac{1}{4}$ | $\frac{2}{3}$ | 85<br>20       | 2.9 I<br>2.9 F | 0.25                       | 0.5            | 1.96     |      |             |         |          |

Scrub 1st Rougher for 5 minutes at 20% solids with 2.0 lb./ton NaOH, deslime and wash

|                        |                 |               |                |  |  |  |      |     |     |      |
|------------------------|-----------------|---------------|----------------|--|--|--|------|-----|-----|------|
| 1st Zircon Concentrate | { $\frac{1}{4}$ | $\frac{2}{3}$ | 9.5 I          |  |  |  | 0.08 | 2.0 | 0.2 | 0.17 |
| 2nd Zircon Concentrate | { $\frac{1}{4}$ | 1             | 9.2 I<br>6.9 F |  |  |  | 0.04 |     | 0.2 | 0.17 |

REMARKS.—Di-sodium alpha sulfo stearate was prepared in situ by conditioning the ore first with alpha-sulfo stearic acid and then treating the ore with a stoichiometric amount of sodium hydroxide to neutralize the acid. Crude fuel oil used is No. 6 grade Bunker "C" fuel oil. Starch 3366 is a corn starch obtained from Corn Products, 1st and 2nd Zircon concentrates combined for analysis. Armac T is an acetate salt of a tallow amine.

## METALLURGICAL RESULTS

| Product                  | Weight, Grams | Weight, Percent | Percent Heavy Minerals | Percent Grade | Percent Recovery |
|--------------------------|---------------|-----------------|------------------------|---------------|------------------|
| Quartz Conc.             | 174           | 34.8            | 16.27                  |               |                  |
| Zircon Conc.             | 168           | 33.5            | 98.80                  | 66.0          | 91.2             |
| Aluminum Silicates Conc. | 158           | 31.7            | 99.24                  | 94.3          | 65.0             |
|                          | 500           |                 |                        |               |                  |

## Remarks

The ore used in the tests conducted was the resultant nonconductor, non-magnetic product from electrostatic separation and separation over induced roll magnets. The electrostatic separation removed the ilmenite and rutile while the induced roll magnets removed the staurolite and dumortierite leaving an aluminum silicates-zircon-quartz fraction. This had an approximate composition of 45% aluminum silicates, 25% zircon and 30% quartz. Compositions on this and on subsequent products obtained by flotation were determined by a petrographic analysis. Heavy mineral analysis was determined by a heavy media separation.

The analyses indicate an upgrading of minerals in both the aluminum silicates concentrate and the zircon concentrate. Percent heavy minerals essentially is the total heavy mineral grade in each product obtained, with the remainder consisting of quartz. Percent grade indicates the grade of the mineral being concentrated, taking into account both the quartz and other heavy minerals as contaminants. Percent recovery represents that portion of the total mineral appearing in the particular product that is considered to be the concentrate.

We claim:

1. A process for the concentration of quartz, aluminum silicate and zircon from a non-conductive non-magnetic fraction of beach sand concentrate, comprising floating the aluminum silicates and zircon away from the quartz particles in a first aqueous medium containing a fluorine-containing acid and an anionic collector selected from the group consisting of alpha sulfo fatty acids, the alkali metal salts of such acids, the glycerol and glycol esters of the acids, sulfonated oils and the alkali metal salts of such oils, said first aqueous medium having been adjusted to a pH not exceeding 6.0 for said flotation step, removing the aluminum silicates and zircon in the overflow, chemically treating the aluminum silicates and zircon to remove the collector, and separating the zircon

40 3. The process, as claimed in claim 1 wherein the anionic collector is alpha sulfo palmitic acid.

4. The process, as claimed in claim 1 wherein the anionic collector is monoethylene glycol ester of alpha sulfo stearic acid.

5 5. The process, as claimed in claim 1 wherein the anionic collector is the monoethylene glycol ester of alpha sulfo palmitic acid.

6 6. A process for the concentration of quartz, the kyanite-sillimanite and the zircon from a non-conductive, non-magnetic fraction of beach sand concentrate, comprising floating the kyanite-sillimanite and zircon away from the quartz particles in a first aqueous medium containing hydrofluoric acid and alpha sulfo stearic acid, said first aqueous medium having been adjusted to a pH not exceeding 6.0 for said flotation step, removing the kyanite-sillimanite and zircon in the overflow and separating the zircon from the kyanite-sillimanite in a second aqueous medium containing an amine collector and a depressant selected from the group consisting of dextrans, gums and starches, said second aqueous medium having been adjusted to a pH of from 7.0 to 12.0 for said separation.

60 References Cited in the file of this patent

## UNITED STATES PATENTS

|           |                |               |
|-----------|----------------|---------------|
| 2,082,383 | Corbett        | June 1, 1937  |
| 2,185,541 | Cahn           | Jan. 2, 1940  |
| 2,205,503 | Trotter        | June 25, 1940 |
| 2,305,502 | Tartaron       | Dec. 15, 1942 |
| 2,341,046 | Kirby          | Feb. 9, 1944  |
| 2,414,815 | Kennedy et al. | Jan. 28, 1947 |
| 2,459,219 | Duke           | Jan. 18, 1949 |
| 2,460,968 | Bert           | Feb. 8, 1949  |
| 2,792,940 | Baarson        | May 21, 1957  |
| 2,970,688 | Uhland         | Feb. 7, 1961  |
| 3,008,655 | Adams et al.   | Nov. 14, 1961 |

## FOREIGN PATENTS

|         |        |              |
|---------|--------|--------------|
| 479,072 | Canada | Dec. 4, 1951 |
|---------|--------|--------------|